

# UNITED STATES PATENT OFFICE.

ALFRED SCHWARZ, OF JOPLIN, MISSOURI, ASSIGNOR TO METALS RECOVERY COMPANY, OF NEW YORK, N. Y., A CORPORATION OF MAINE.

## COMPOSITION AND SUBSTANCE FOR USE IN CONCENTRATION OF ORES AND METHOD OF PRODUCING SAME.

1,427,232.

Specification of Letters Patent. Patented Aug. 29, 1922.

No Drawing. Application filed March 6, 1917, Serial No. 152,586. Renewed June 1, 1922. Serial No. 565,128.

*To all whom it may concern:*

Be it known that I, ALFRED SCHWARZ, a subject of the Emperor of Germany, residing in Joplin, county of Jasper, State of Missouri, have invented certain new and useful Improvements in Compositions and Substances for Use in the Concentration of Ores and Methods of Producing Same; and I do hereby declare the following to be a full, 10 clear, and exact description of the invention, such as will enable others skilled in the art to which it appertains to make and use the same.

This invention relates to compositions or 15 substances or agents adapted for use in the concentration of ores and to the method of producing such compositions and the like.

In my companion application Serial No. 152,585 filed March 6, 1917, I have described 20 and claimed a process of concentrating ores and the like by the use of such compositions and substances and agents as those referred to. The present invention relates more particularly to such compositions and substances 25 themselves and to the method of their production.

Heretofore various methods of concentrating ores have been proposed for the removal or separation of mineral constituents 30 therefrom by the use of selective agents, such as oils, oily substances, resinous substances, various mixtures of oils, and the like. The oils or other substances used have generally been those which are available commercially 35 in sufficient amounts and at a sufficiently low cost; and they have been largely products from distillation processes or by-products of other industrial processes.

In the practice of flotation processes heretofore carried on, it has been customary to 40 use flotation agents in the form in which they are commercially available and to compound those agents in various proportions in an endeavor to produce a composite product 45 which will give satisfactory results with the particular ore to be treated. Such procedures involve the use of all the constituents of the oily or other substances, including both the soluble and extractable, as well as 50 the insoluble or immiscible constituents.

Where the selective agents have contained considerable amounts of insoluble or immiscible constituents it has been the practice, as

above stated, to effect an intimate disintegration or breaking up of the oily substance, 55 as by "emulsification" thereof with the water or ore pulp, in order that effective action might be secured. In such procedures, however, there is involved the indiscriminate use of all the constituents present 60 in the oily substance in question.

The selective agents commonly used in ore concentration have been generally classed either as insoluble and immiscible substances, such as many of the common oils, 65 or as soluble substances or frothing agents.

I have found, however, as the result of careful experimentation, that the so-called insoluble or immiscible oils are nevertheless under the conditions of their present use, 70 soluble to a certain extent, or contain soluble constituents, and that it is largely to such soluble constituents that the concentrating action is due. Moreover, the so-called soluble frothing agents which are 75 available commercially, nevertheless contain insoluble or immiscible constituents. Where such insoluble or immiscible constituents are present in association with the soluble or extractable constituents, the action of the 80 soluble or extractable constituents is masked or inhibited. Not only is it usually necessary to break up the oily substance to an extent sufficient to disclose and set free the soluble constituents, but the insoluble or immiscible constituents themselves may even be 85 injurious to the flotation process.

According to the present invention, these uncertainties and disadvantages are largely overcome or minimized. I have found that 90 by subjecting various selective agents, including many substances of an oily or resinous nature, to an extraction process with aqueous extracting liquors, and by separating the extracted constituents from the unextracted constituents, and by using the thus extracted constituents, either with or without the addition thereto, in predetermined amounts, of the unextracted constituents, 95 it is possible to obtain higher grade concentrates and a better separation generally; and that it is thus possible to effect the concentration of ores with greater reliability than heretofore usually possible.

I may take an impure product, for instance, products of distillation such as

crude creosote, coal tar, pine tar, rosin, rosin oil and many others, and extract from the same, by a simple and inexpensive treatment, concentrating agents giving more definite and clearer separation than has been obtained with the substances now in use. Furthermore, selective agents solid at normal temperature may be obtained and used in ore concentrating methods with cold water, and in a form in which they are freed from injurious impurities.

It is accordingly an object of my invention to produce from normally solid substances (rosin, tar, etc.), as well as from liquid substances (oils, etc.), substances suited for use for ore concentration at ordinary temperatures.

I am aware that it has been proposed to utilize for flotation purposes, certain chemical substances which are stated to be completely soluble, but so far as I am aware, no such processes are commercially feasible because of the prohibitive cost of the isolated chemical individuals which it is thus proposed to use.

The commercial utilization of the so-called soluble selective agents has involved the accompanying use of their insoluble constituents, the action thus partaking of the action of the so-called insoluble oils which nevertheless also contain soluble constituents.

According to the present invention, the selective agents (for example rosin, pine-tar, pine oil, coal tar and its distillates, etc.) are subjected to a disintegration and extraction in water or like aqueous liquor, so that there are separated the soluble or extractable constituents from the insoluble or immiscible constituents. This disintegration and extraction may be effected by agitating with cold or hot water, or by boiling with water, or with dilute alkaline or acid liquors. Again the selective agents, for example rosin, or certain pine oil or pine tar or coal tar products, may be subjected to an extraction with alkali liquors and the extracted constituents subsequently treated with acids to remove constituents therefrom which are insoluble in dilute acids. Various methods of extraction can be used for disintegrating the selective agents and separating the extractable from the non-extractable constituents. So also, as where dilute alkalies are used, there may be extracted first all constituents soluble in the dilute alkalies and the remaining insoluble constituents separated; after which there is effected a further separation from the alkali solution all those constituents which are insoluble in acids. Where the solutions obtained contain constituents injurious to the concentration operation, they may be purified or treated in order to remove such injurious constituents therefrom.

The selective agents which are available for treatment according to the present invention to produce the new compositions or substances, include most, and I believe all, of the selective agents and the like which are commonly used in flotation methods of concentration. These will, however, vary considerably in their value and in the amount of extractable constituents which they yield. Where, however, there remain considerable amounts of insoluble constituents, and where a part only, and often a small part, of the insoluble constituents are desired for use in the concentration of ores, along with the extracted constituents, the remainder of the insoluble constituents may be diverted to other purposes, thus reducing materially the cost of the concentration process. Inasmuch as but relatively small amounts of the novel compositions or substances are usually necessary for the concentration of ores, even as compared with the amounts of "oils" commonly used, it will be evident that in many cases, there will be produced a very considerable amount of material rejected from this particular process and available for other purposes, this material being of relatively little or no value or a detriment for use in the concentration of ores.

It may be advantageous in some cases, to completely dissolve the substance treated, when soluble, as in dilute alkalies, and to re-precipitate the dissolved constituents insoluble in water or in dilute acids, as by adding acids, in order that the soluble constituents distributed throughout the original mass may be set free and rendered available.

The various substances treated, after extraction, are adapted for use for other purposes, where they are not required for ore concentrating purposes, e. g., for use in water-proofing compositions, and in such case they may even be of enhanced value because of the removal therefrom of the soluble or extractable constituents, since for many purposes the soluble or extractable constituents are undesirable and even detrimental.

Instead of extracting the selective agents themselves, certain raw materials and sources thereof may be directly extracted, such as certain wood fibres and plants or bituminous substances which form sources of oils, resins, etc.

The invention will be further illustrated by the following more detailed description of certain embodiments thereof. For example, using rosin as the raw material, it may be disintegrated or broken up and extracted in various ways. It may thus be subjected to the action of boiling water, the mass being constantly agitated by any suitable means. After such portions of the rosin as are soluble have come into solution,

or after such portions as are desired to extract, have been extracted, the mass is filtered or otherwise treated to separate the original constituents. The soluble constituents are available for use directly in the concentration of ores or they may be re-combined with predetermined amounts of the insoluble constituents. So also the extracted constituents may be concentrated as 5 by evaporation to produce a more concentrated solution or even solids. Again any of the extracted components of one material may be compounded with any number of extracted components of another material. Where the extraction of rosin is carried out so that the extracted portions contain constituents precipitated with acids or alkalies, such substances may be precipitated and the resulting solutions used either alone 10 or with the addition of the precipitated substances in predetermined amount. The amount to be so added can be readily determined by a simple experiment or experiments with the particular ore pulp in question.

As another instance, rosin may be subjected to a solution of one percent sodium hydroxide until the soluble portions have been taken into solution. The mass may, if desired, be treated with substances reacting with tannic acid, gum or other constituents which may be desirable to remove. Separation of the solution is thereafter effected by decantation, filtration or other means and the solution is then treated with a small amount of a suitable acid which may be sufficient to neutralize all or part of the alkali or even to make the solution acid with an excess of acid. Any precipitate thus formed may or may not be thus separated. By separating the precipitate, the solution can be used by itself or it can be used with predetermined amounts of the precipitate or of other constituents.

45 The invention will be further illustrated by the following instance of its application: Forty parts by weight of common pine rosin are boiled with two thousand parts of water containing forty parts of caustic soda dissolved therein. Forty parts of litharge or its equivalent in lead acetate are added after the rosin is in solution and the mixture is maintained hot for about two hours. The solution is then filtered off, preferably hot, 50 and any desired portion of the solution is then subjected to treatment with sulfuric acid. Assuming that thirty parts of the mixture is to be used with five hundred parts by weight of ore (greater or less proportions, however, are effective), the thirty parts of the liquor are acidified with three parts of ten percent sulfuric acid solution which causes the precipitation of some of the rosin constituents previously in solution, the precipitate is filtered off and the filtrate is then

added to the five hundred parts of ore which is first mixed with two thousand parts of water and the mixture is subjected to a flotation operation of concentration.

It will be evident that various methods of concentration can be carried out with the compositions and agents of the present invention and in referring to a particular example of how such agents may be used, I do so merely by way of illustration. The 70 compositions produced according to the present invention may be supplied in various ways for use in such ore concentrating processes. They may thus be supplied in the form of various concentrations containing 80 predetermined amounts of the components, of any number of original materials used in their production. Again, the agents may be supplied in the form of two or more substances to be mixed by the user previous to, 85 or at the time of, their addition to the ore pulp, or each used separately, as the case may require. Since it is one of the characteristics of the invention that the soluble constituents are separated from the insoluble 90 constituents, advantage may be taken of this by the operator by adding any of the various separated components in any desired rotation or sequence or combination best suited to obtaining the desired results.

95 For an ore containing considerable amounts of colloidal or finely divided gangue it is usually desirable to use a predominating amount of the soluble compositions or agents because of the tendency of 100 the insoluble constituents to adhere to such gangue constituents; whereas with coarser ores or ores relatively free from colloidal and finely divided gangue, it is usually desirable to have predetermined amounts of 105 the insoluble constituents present, e. g. to form a more coherent froth. The compositions and agents of the present invention can accordingly be supplied for the particular ore to be concentrated, the nature of 110 the composition depending particularly, as to its presence or absence of insoluble constituents, upon the nature of the ore and particularly upon the presence or absence and amount of colloidal or finely divided 115 gangue.

Instead of extracting from different raw materials the extractable constituents, and thereafter combining the same, the raw materials may be combined before extraction and a composite extract thereby produced. The extraction in such cases may be effected by agitation with hot or cold water or by other suitable means for separating or extracting the soluble constituents 120 from those which are insoluble; and in this case also the composition or agent to be subsequently used may be formed of either the soluble constituents or a combination thereof 125 with predetermined amounts of insoluble 130

4 constituents. The raw materials to be treated may, as previously stated, be of either liquid or solid consistency and of vegetable, animal or mineral origin, provided that they contain extractable constituents of the nature indicated, I have found that rosin is of particular value as a raw material for the production of flotation agents. So also pine tar and pine oil are 10 of value, as is also creosote. Crude oil is of relatively less value in that much larger amounts of it are required for the production of sufficient amounts of flotation agents as compared, for example, with rosin or 15 pine oil. Whereas the use of the common oils and oil mixtures (such as are commonly used in flotation) involves the use of all the insoluble constituents carried by the oils, with the results that the insoluble constituents are usually present in amounts having no relation to the amount necessary or desirable, the novel compositions of the 20 present invention enabling the ore to be concentrated either with the soluble or extracted constituents alone, or with such added amounts of insoluble constituents as may be predetermined for the particular ore under treatment.

In the foregoing description and in the 30 accompanying claims, I use the term "selective agents" as a generic term to include the various substances, such as oil, resins, tars and the like.

I claim:

35 1. The method of producing agents and compositions for use in the concentration of ores, which comprises disintegrating selec-

tive agents by extraction first with an aqueous alkali, removing any unextracted constituents treating with an acid and removing 40 any separated solid constituents, and thereby obtaining a solution containing soluble constituents and freed from constituents insoluble in the alkali and acid together with other components or constituents utilizable 45 separately or in combination with each other.

2. The method of producing agents and compositions for use in the concentration of ores, which comprises extracting selective agents containing insoluble constituents by 50 agitation with an alkaline liquor, separating the resulting extracted constituents from the insoluble residue, neutralizing the alkaline solution with acid and thereby precipitating constituents insoluble in acid, 55 separating the resulting solution from the precipitate and thereby obtaining a solution freed from constituents insoluble in the alkali and acid; substantially as described.

3. The method of producing agents and compositions for use in the concentration of ores, which comprises extracting resins with an alkaline liquor, separating the unextracted constituents from the resulting solution, treating the solution with an acid and removing any separated solid constituents, and thereby obtaining a solution containing soluble constituents together with separate insoluble components or constituents utilizable 60 separately or in combination with each other.

In testimony whereof, I affix my signature.

ALFRED SCHWARZ.